# EUROPEAN PATENT SPECIFICATION

(11) **EP 2 088 881 B1**
(45) Date of publication and mention of the grant of the patent: **31.12.2014**
(21) Application number: 07839908.6
(22) Date of filing: 02.11.2007
(51) Int. Cl.: A41D 31/02, D04H 13/00

(54) **OUTERWARE GARMENT COMPRISING A BREATHABLE WATERPROOF FABRIC WITH A DYED AND WELDED MICROPOROUS LAYER**
OBERBEKLEIDUNG MIT EINEM ATMUNGSAKTIVEN, WASSERDICHTEN STOFF MIT EINER GEFÄRBTEN UND GESCHWEISSTEN MIKROPORÖSEN LAGE
VETEMENT DE DESSUS AVEC UN TISSU IMPERMEABLE RESPIRANTS AVEC UNE COUCHE TEINTE ET SOUDEE A MICROPORES

(30) Priority: 03.11.2006 US 856516 P
(43) Date of publication of application: 19.08.2009
(73) Proprietor: E.I. DU PONT DE NEMOURS AND COMPANY, Wilmington, DE 19898 (US)
(72) Inventor: CONLEY, Jill A., Midlothian, VA 23112 (US); GUCKERT, Joseph Robert, Chester, VA 23836 (US); MARIN, Robert Anthony, Midlothian, VA 23114 (US); PALMER, George Bruce IV, Richmond, VA 23221 (US)
(74) Representative: Morf, Jan Stefan
(86) International application number: PCT/US2007/023144
(87) International publication number: WO 2008/057417

(56) References cited:
- EP-A- 1 364 773
- WO-A-01/27368
- WO-A-97/46750
- WO-A-2004/027140
- WO-A-2005/103354
- WO-A-2006/049664
- WO-A-2008/021293

## Description

### FIELD OF THE INVENTION

This invention relates to outer ware garments incorporating a multi-layer moisture and water management fabric.

### BACKGROUND OF THE INVENTION

Protective garments for wear in rain and other wet conditions should keep the wearer dry by preventing the leakage of water into the garment and by allowing perspiration to evaporate from the wearer to the atmosphere. "Breathable" materials that do permit evaporation of perspiration have tended to wet through from the rain, and they are not truly waterproof. Oilskins, polyurethane coated fabrics, polyvinyl chloride films and other materials are waterproof but do not allow satisfactory evaporation of perspiration.

Fabrics treated with silicone, fluorocarbon, and other water repellants usually allow evaporation of perspiration but are only marginally waterproof; they allow water to leak through under very low pressures and usually leak spontaneously when rubbed or mechanically flexed. Rain garments must withstand the impingement pressure of falling and wind blown rain and the pressures that are generated in folds and creases in the garment.

It is widely recognized that garments must be "breathable" to be comfortable. Two factors that contribute to the level of comfort of a garment include the amount of air that does or does not pass through a garment as well as the amount of perspiration transmitted from inside to outside so that the undergarments do not become wet and so that the natural evaporative cooling effect can be achieved. However even recent developments in breathable fabric articles using microporous films tend to limit moisture vapor transmission if air permeability is to be controlled.

Many waterproof structures currently available comprise a multilayer fabric structure that employs the use of a hydrophobic coating. This fabric structure is typically made of a woven fabric layer, a membrane-type microporous layer, and another woven layer. The microporous layer is the functional layer of the construction that provides the appropriate air permeability and moisture vapor transmission rate necessary for the targeted application. For examples of such structures see U.S. patent numbers 5,217,782; 4,535,008; 4,560,611 and 5,204,156.

The material currently in use in many waterproof and/or windproof breathable garments is an expanded PTFE (e-PTFE) microporous structure that is white in color. This material cannot be dyed and therefore produces a white edge when cut and sewn into a garment. This white edge is not acceptable in the higher-end market applications to which this microporous structure is targeted. Post-processing steps to hide the white edge must be included in the final construction of any fabric structure containing the e-PTFE.

Additionally, the chemical nature of this material is such that the edges, zippers, pockets, etc. of any fabric structure containing the e-PTFE must be stitched. This stitching causes the fabrics windproof and/or waterproof functionality to weaken at that point, and additional post-processing must be applied to the stitched area in order to regain the waterproof/windproof functionality.

EP 13 64 773 A1 discloses an outer ware garment with a microporous layer of polymeric fibers.

What is needed is a microporous layer that can be dyed to match the color of the other layers in the fabric structure. This coloring can be done either during or after the production of the submicron nonwoven structure. This coloring of the microporous layer will omit any post-processing step that is done to hide a white edge.

What is also needed is a microporous layer that can be thermally bonded in order to eliminate the stitching in a fabric structure. This thermal bonding will create a completely seam-free waterproof and/or windproof structure and will eliminate any post-processing that must be done at the site of a seam in order to regain the waterproof and/or windproof functionality of a fabric structure.

While it is well known for example that e-PTFE is a desirable material for use in waterproof breathable and wind barrier fabrics in garments, the high temperature melting point and other negative aspects of e-PTFE mean that it does not readily melt at the same temperature as common textile materials such as nylon or polyester. In garments it is increasingly desirable to seam seal by thermal or ultrasonic welding techniques.

These techniques depend on the melting temperature of the materials involved. Lower melting temperatures are more amenable to these techniques. In addition, similar melting characteristics of multicomponent structures are more desirable so that the materials combine more properly within the weld.

In order to thermally seam weld multicomponent fabric structures including e-PTFE it is necessary to overcome these issues created by the dissimilar high melting temperatures of e-PTFE. To do this a more complex seam welding technique is used called "feld-seaming", which involves multiple folds of the structure to allow face fabric to face fabric contact and welding. This creates a thicker and heavier seam, which is not desirable for aesthetics and comfort. In addition, to create the feld-seam a special fitting must be attached to the seam welding machine. This may also be slower and more prone to processing errors/waste than conventional seaming without the presence of e-PTFE. In addition the process of seam welding and raising the temperature of the e-PTFE can lead to "fractures" within the e-PTFE, which can lead to failures in the final garment.

The present invention is directed towards a layered material for a garment that provides controlled liquid water resistance in the presence of high vapor transmittance and is hence highly waterproof and is also dyeable and weldable.

### SUMMARY OF THE INVENTION

The invention is directed to an outerware garment having the ability to pass moisture vapor while protecting the wearer from wind and liquid water comprising a composite fabric of at least one fabric layer adjacent to and in a face-to-face relationship with a dyeable nanofiber layer, wherein the nanofiber layer comprises at least one microporous layer of polymeric nanofibers having a number average diameter between 50 nm and less than 1000 nm, and a basis weight of between 1 g/m² and 100 g/m², wherein the composite fabric has a Frazier air permeability of between 1.2 m³/m²/min and 7.6 m³/m² /min, and an MVTR per ASTM E-96B of greater than about 500 g/m² /day, and said nanofiber layer being welded to the fabric layer over some fraction of its surface.

### DETAILED DESCRIPTION

In one embodiment the invention comprises a nanofiber layer adjacent to a fabric layer and optionally bonded thereto over at least a fraction of its surface. The terms "nanofiber layer" and "nanoweb" are used interchangeably herein.

The term "nanofiber" as used herein refers to fibers having a number average diameter or cross-section less than about 1000 nm, even less than about 800 nm, even between about 50 nm and 500 nm, and even between about 100 and 400 nm. The term diameter as used herein includes the greatest cross-section of non-round shapes.

The term "nonwoven" means a web including a multitude of randomly distributed fibers. The fibers generally can be bonded to each other or can be unbonded. The fibers can be staple fibers or continuous fibers. The fibers can comprise a single material or a multitude of materials, either as a combination of different fibers or as a combination of similar fibers each comprised of different materials.

"Meltblown fibers" are fibers formed by extruding a molten thermoplastic material through a plurality of fine, usually circular, die capillaries as molten threads or filaments into converging, usually hot and

high velocity, gas, e.g. air, streams to attenuate the filaments of molten thermoplastic material and form fibers. During the meltblowing process, the diameter of the molten filaments is reduced by the drawing air to a desired size. Thereafter, the meltblown fibers are carried by the high velocity gas stream and are deposited on a collecting surface to form a web of randomly disbursed meltblown fibers. Such a process is disclosed, for example, in U.S. Pat. Nos. 3,849,241 to Buntin et al., 4,526,733 to Lau, and 5,160,746 to Dodge, II et al.. Meltblown fibers may be continuous or discontinuous.

"Calendering" is the process of passing a web through a nip between two rolls. The rolls may be in contact with each other, or there may be a fixed or variable gap between the roll surfaces. Advantageously, in the present calendering process, the nip is formed between a soft roll and a hard roll. The "soft roll" is a roll that deforms under the pressure applied to keep two rolls in a calender together. The "hard roll" is a roll with a surface in which no deformation that has a significant effect on the process or product occurs under the pressure of the process. An "unpatterned" roll is one which has a smooth surface within the capability of the process used to manufacture them. There are no points or patterns to deliberately produce a pattern on the web as it passed through the nip, unlike a point bonding roll.

In one embodiment, the invention is directed to a breathable fabric having the ability to maintain a high MVTR while comprising a microporous layer that can be dyed and/or welded to the other fabrics in a garment. The fabric comprises a nanofiber layer that in turn comprises at least one porous layer of polymeric nanofibers having a basis weight of between about 1 g/m² and about 100 g/m².

The invention further comprises a first fabric layer adjacent to and in a face-to-face relationship with the nanofiber layer and optionally further comprises a second fabric layer adjacent to and in a face-to-face relationship with the nanofiber layer and on the opposite side of the nanofiber layer to the first fabric layer.

The barrier fabric of the invention further has a Frazier air permeability of between about 1.2 m³/m²/min and about 7.6 m³/m²/min, and an MVTR per ASTM E-96B method of greater than about 500 g/m²/day.

The nonwoven web may comprise primarily or exclusively nanofibers that are produced by electrospinning, such as classical electrospinning or electroblowing, and in certain circumstances by meltblowing processes. Classical electrospinning is a technique illustrated in U.S. Patent No. 4,127,706, wherein a high voltage is applied to a polymer in solution to create nanofibers and nonwoven mats. The nonwoven web may also comprise melt blown fibers.

The "electroblowing" process for producing nanowebs is disclosed in World Patent Publication No. WO 03/080905. A stream of polymeric solution comprising a polymer and a solvent is fed from a storage tank to a series of spinning nozzles within a spinneret, to which a high voltage is applied and through which the polymeric solution is discharged. Meanwhile, compressed air that is optionally heated is issued from air nozzles disposed in the sides of or at the periphery of the spinning nozzle. The air is directed generally downward as a blowing gas stream which envelopes and forwards the newly issued polymeric solution and aids in the formation of the fibrous web, which is collected on a grounded porous collection belt above a vacuum chamber. The electroblowing process permits formation of commercial sizes and quantities of nanowebs at basis weights in excess of about 1 gsm, even as high as about 40 gsm or greater, in a relatively short time period.

The fabric component of the invention can be arranged on the collector to collect and combine the nanoweb spun on the fabric, so that the combined fiber web is used as the fabric of the invention.

Polymer materials that can be used in forming the nanowebs of the invention are not particularly limited and include both addition polymer and condensation polymer materials such as, polyacetal, polyamide, polyester, cellulose ether and ester, polyalkylene sulfide, polyarylene oxide, polysulfone, modified polysulfone polymers and mixtures thereof. Preferred materials that fall within these generic classes include, poly(vinylchloride), polymethylmethacrylate (and other acrylic resins), polystyrene, and copolymers thereof (including ABA type block copolymers), poly(vinylidene fluoride), poly(vinylidene chloride), polyvinylalcohol in various degrees of hydrolysis (87% to 99.5%) in crosslinked and non-crosslinked forms. Preferred addition polymers tend to be glassy (a T_{g} greater than room temperature). This is the case for polyvinylchloride and polymethylmethacrylate, polystyrene polymer compositions or alloys or low in crystallinity for polyvinylidene fluoride and polyvinylalcohol materials. One preferred class of polyamide condensation polymers are nylon materials, such as nylon-6, nylon-6,6, nylon 6,6-6,10 and the like. When the polymer nanowebs of the invention are formed by meltblowing, any thermoplastic polymer capable of being meltblown into nanofibers can be used, including polyolefins, such as polyethylene, polypropylene and polybutylene, polyesters such as poly(ethylene terephthalate) and polyamides, such as the nylon polymers listed above.

The as-spun nanoweb of the present invention can be calendered in order to impart the desired physical properties to the fabric of the invention, as disclosed in co-pending U.S. Patent Application No. 11/523,827, filed September 20, 2006. The as-spun nanoweb can be fed into the nip between two unpatterned rolls in which one roll is an unpatterned soft roll and one roll is an unpatterned hard roll, and the temperature of the hard roll is maintained at a temperature that is between the T_{g}, herein defined as the temperature at which the polymer undergoes a transition from glassy to rubbery state, and the Tₒₘ, herein defined as the temperature of the onset of melting of the polymer, such that the nanofibers of the nanoweb are at a plasticized state when passing through the calendar nip. The composition and hardness of the rolls can be varied to yield the desired end use properties of the fabric. One roll can be a hard metal, such as stainless steel, and the other a soft-metal or polymer-coated roll or a composite roll having a hardness less than Rockwell B 70. The residence time of the web in the nip between the two rolls is controlled by the line speed of the web, preferably between about 1 m/min and about 50 m/min, and the footprint between the two rolls is the MD distance that the web travels in contact with both rolls simultaneously. The footprint is controlled by the pressure exerted at the nip between the two rolls and is measured generally in force per linear CD dimension of roll, and is preferably between about 1 mm and about 30 mm.

Further, the nanoweb can be stretched, optionally while being heated to a temperature that is between the T_{g} and the lowest Tₒₘ of the nanofiber polymer. The stretching can take place either before and/or after the web is fed to the calender rolls and in either or both the machine direction or cross direction.

A wide variety of natural and synthetic fabrics are known and may be used as the fabric layer or layers in the present invention, for example, for constructing garments, such as sportswear, rugged outerwear and outdoor gear, protective clothing, etc. (for example, gloves, aprons, chaps, pants, boots, gators, shirts, jackets, coats, socks, shoes, undergarments, vests, waders, hats, gauntlets, sleeping bags, tents, etc.). Typically, vestments designed for use as rugged outerwear have been constructed of relatively loosely-woven fabrics made from natural and/or synthetic fibers having a relatively low strength or tenacity (for example, nylon, cotton, wool, silk, polyester, polyacrylic, polyolefin, etc.). Each fiber can have a tensile strength or tenacity of less than about 8 g/Denier (gpd), more typically less than about 5 gpd, and in some cases below about 3 gpd. Such materials can have a variety of beneficial properties, for example, dyeability, breathability, lightness, comfort, and in some instances, abrasion-resistance.

Different weaving structures and different weaving densities may be used to provide several alternative woven composite fabrics as a component of the invention. Weaving structures such as plain woven structures, reinforced plain woven structures (with double or multiple warps and/or wefts), twill woven structures, reinforced twill woven structures (with double or multiple warps and/or wefts), satin woven structures, reinforced satin woven structures (with double or multiple warps and/or wefts), knits, felts, fleeces and needlepunched structures may be used. Stretch woven, ripstops, dobby weaves, jacquard weaves, are also suitable for use in the present invention.

The nanoweb is welded to the fabric layers over some fraction of its surface and can be welded to the fabric layer by any means known to one skilled in the art, for example thermally, optionally using an ultrasonic field.

"Welding means" in the context of this invention refers to the manner in which lamination of two webs into a composite structure is accomplished. Methods that are suitable in the context of this invention are exemplified by, but not limited to, ultrasonic bonding and point bonding. Those skilled in the art are familiar with the various types of welding, and are capable of adapting any suitable welding means for use in the invention.

Ultrasonic bonding for example typically entails a process performed, for example, by passing a material between a sonic horn and an anvil roll such as illustrated in U.S. Pat. Nos. 4,374,888 and 5,591,278. In an exemplary method of ultrasonic bonding, the various layers that are to be attached together are simultaneously fed to the bonding nip of an ultrasonic unit. A variety of these units are available commercially. In general, these units produce high frequency vibration energy that melt thermoplastic components at the bond sites within the layers and join them together. Therefore, the amount of induced energy, speed by which the combined components pass through the nip, gap at the nip, as well as the number of bond sites determine the extent of adhesion between the various layers. Very high frequencies are obtainable, and frequencies in excess of 18,000 Hz (cycles per second) are usually referred to as ultrasonic, depending on the desired adhesion between various layers and the choice of material, frequencies as low as 5,000 Hz or even lower may produce an acceptable product.

The invention will now be illustrated by the following specific examples:

### Examples

In Example 1 a three-layer fabric construction was made from a nylon ripstop (basis weight 100 gsm), a nanoweb made from Nylon 6,6, and a nylon mesh material using a solvent-based urethane adhesive using a "288-pattern" gravure-roll application with a pressure of 60 psi.

In Example 2, a three-layer fabric construction was made from a nylon ripstop (basis weight 100 gsm), a nanoweb made from Nylon 6,6, and a nylon tricot material (basis weight 35 gsm) using a solvent-based urethane adhesive using a "288-pattern" gravure-roll application with a pressure of 60 psi. The final three-layer constructions were then ultrasonically bonded using SeamMaster™ with various stitch types, to include flat, reinforced, and curved stitching.

The constructions from Examples 1 and 2 were then tested for breaking strength, elongation at maximum load, percent elongation at break, modulus, tensile strength, and energy at maximum load using an Instron™ tensile machine with samples 25.40mm wide. The load cell used was 5kN. Also tested were single-stitch seams from a Zero Resistance® Golf Outerwear vest. The results are indicated in the table.

| Sample | Breaking Strength Ibf/in | Elongation at max load % | Elongation at break % |
|---|---|---|---|
| Golf outerwear vest (control) | 21.16 | 7.43 | 7.48 |
| Example 1 | 9.58 | 21.76 | 23.64 |
| Example 2 | 9.23 | 51.82 | 58.8 |

As the data show, the breaking strength of an ultrasonically bonded seam is roughly half that of a single-stitch seam. These are very good results and show that ultrasonically bonding a fabric construction has the potential to replace single-stitch seams, thus eliminating the need for the extra step of applying seam tape to a stitch.

## Claims

1. An outerware garment having the ability to pass moisture vapor while protecting the wearer from wind and liquid water comprising a composite fabric of at least one fabric layer adjacent to and in a face-to-face relationship with a dyeable nanofiber layer, wherein the nanofiber layer comprises at least one microporous layer of polymeric nanofibers having a number average diameter between 50 nm and less than 1000 nm, and a basis weight of between 1 g/m² and 100 g/m², wherein the composite fabric has a Frazier air permeability of between 1.2 m³/m²/min and 7.6 m³/m² /min, and an MVTR per ASTM E-96B of greater than about 500 g/m² /day, and said nanofiber layer being welded to the fabric layer over some fraction of its surface.

2. The garment of claim 1 in which the nanofiber layer comprises polymer from a class selected from the group consisting of polyacetals, polyamides, polyesters, cellulose ethers, cellulose esters, polyalkylene sulfides, polyarylene oxides, polysulfones, modified polysulfone polymers and mixtures thereof.

3. The garment of claim 1 in which the nanofiber layer comprises polymer from the group consisting of poly(vinylchloride), polymethylmethacrylate, polystyrene, and copolymers thereof, polyvinylalcohol in crosslinked and non-crosslinked forms.

4. The garment of claim 2 in which the nanofiber layer comprises polymer from the group consisting of nylon-6, nylon-6,6, nylon 6,6-6,10.

5. The garment of claim 1 in which the first fabric is woven from a material selected from the group consisting of nylon, cotton, wool, silk, polyester, polyacrylic, polyolefin and combinations thereof.

6. The garment of claim 1 in which the first fabric is woven from fibers that have a tenacity of less than about 8 g/Denier (gpd).

## Patentansprüche

1. Oberbekleidung, die die Fähigkeit besitzt, Feuchtigkeitsdampf hindurch zu lassen, während sie den Träger gegen Wind und flüssiges Wasser schützt, umfassend einen Verbundtextilstoff aus mindestens einer Textilstofflage, der an einer färbbaren Nanofaserlage anliegt und sich in einem Oberflächen-zu-Oberflächen-Verhältnis damit befindet, wobei die Nanofaserlage mindestens eine mikroporöse Lage aus polymeren Nanofasern umfasst, die einen zahlendurchschnittlichen Durchmesser zwischen 50 nm und weniger als 1000 nm und ein Flächengewicht zwischen 1 g/m² und 100 g/m² aufweisen, wobei der Verbundtextilstoff eine Frazier-Luftdurchlässigkeit zwischen 1,2 m³/m²/min und 7,6 m³/m²/min und eine Feuchtigkeitsdampfdurchlässigkeit (MVTR) ASTM E-96B entsprechend von mehr als etwa 500 g/m²/Tag aufweist, und die Nanofaserlage an die Textilstofflage über einen Teil ihrer Oberfläche geschweißt ist.

2. Kleidungsstück nach Anspruch 1, wobei die Nanofaserlage Polymer aus einer Klasse umfasst ausgewählt aus der Gruppe bestehend aus Polyacetalen, Polyamiden, Polyestern, Celluloseethern, Cellulosestern, Polyalkylensulfiden, Polyarylenoxiden, Polysulfonen, modifizierten Polysulfonpolymeren und Mischung davon.

3. Kleidungsstück nach Anspruch 1, wobei die Nanofaserlage Polymer aus der Gruppe bestehend aus Poly(vinylchlorid), Polymethylmethacrylat, Polystyrol und Copolymeren davon, Polyvinylalkohol in vernetzten und nichtvernetzten Formen umfasst.

4. Kleidungsstück nach Anspruch 2, wobei die Nanofaserlage Polymer aus der Gruppe bestehend aus Nylon-6, Nylon-6,6, Nylon 6,6-6,10 umfasst.

5. Kleidungsstück nach Anspruch 1, wobei der erste Textilstoff aus einem Material gewoben ist ausgewählt aus der Gruppe bestehend aus Nylon, Baumwolle, Wolle, Seide, Polyester, Polyacryl, Polyolefin und Kombinationen davon.

6. Kleidungsstück nach Anspruch 1, wobei der erste Textilstoff aus Fasern gewoben ist, die eine Reißfestigkeit von weniger als etwa 8 g/Denier (gpd) aufweisen.

## Revendications

1. Vêtement de dessus ayant la capacité de laisser passer la vapeur humide tout en protégeant son porteur du vent et de l'eau sous forme liquide comprenant un textile composite d'au moins une couche textile adjacente à, et en relation face à face avec, une couche de nanofibres pouvant être teintées, la couche de nanofibres comprenant au moins une couche microporeuse de nanofibres polymères ayant un diamètre moyen en nombre compris entre 50 nm et inférieur à 1 000 nm, et un poids de base compris entre 1 g/m² et 100 g/m², le textile composite ayant une perméabilité à l'air de Frazier comprise entre 1,2 m³/m²/min et 7,6 m³/m²/min, et un TTVE selon la norme ASTM E-96B supérieur à environ 500 g/m²/jour, et ladite couche de nanofibres étant soudée à la couche textile sur une certaine partie de sa surface.

2. Vêtement selon la revendication 1, dans lequel la couche de nanofibres comprend un polymère d'une classe sélectionnée parmi le groupe constitué des polyacétals, des polyamides, des polyesters, des éthers de cellulose, des esters de cellulose, des poly(sulfures d'alkylène), des poly(oxydes d'arylène), des polysulfones, des polymères de polysulfone modifiés et de leurs mélanges.

3. Vêtement selon la revendication 1, dans lequel la couche de nanofibres comprend un polymère parmi le groupe constitué du poly(chlorure de vinyle), du poly(méthacrylate de méthyle), du polystyrène, et leurs copolymères, du poly(alcool de vinyle) sous des formes réticulées et non réticulées.

4. Vêtement selon la revendication 2, dans lequel la couche de nanofibres comprend un polymère parmi le groupe constitué du nylon-6, du nylon-6,6, du nylon 6,6-6,10.

5. Vêtement selon la revendication 1, dans lequel le premier textile est tissé à partir d'un matériau sélectionné parmi le groupe constitué du nylon, du coton, de la laine, de la soie, du polyester, du polyacrylique, de la polyoléfine et de leurs combinaisons.

6. Vêtement selon la revendication 1, dans lequel le premier textile est tissé à partir de fibres qui présentent une ténacité inférieure à environ 8 g/denier (gpd).
